

## UNITED STATES PATENT OFFICE

GEORGE A. RICHTER, OF BERLIN, NEW HAMPSHIRE, ASSIGNOR TO BROWN COMPANY,  
OF BERLIN, NEW HAMPSHIRE, A CORPORATION OF MAINE

## WHITE WOOD PULP FOR HIGH GRADE PAPER MANUFACTURE

No Drawing.

Application filed November 18, 1930. Serial No. 496,586.

This invention relates to an improved wood pulp derived more especially from kraft pulp and possessing not only the important papermaking characteristics, including 5 strength and tear resistance, of the kraft pulp from which it is derived, but further possessing a pure white color and far greater freedom from resins and ash content and a notably lower pentosan content than is derivation material. The novel product of the 10 present invention is thus one which fulfills the desiderata in two fields of papermaking, namely, that devoted to the manufacture of bond, ledger, and writing papers wherein 15 whiteness of fiber is a prime desideratum, and that devoted to the manufacture of envelope and bag papers, wherein strength and tear resistance are prime desiderata.

Those skilled in the art well know that the 20 conversion of kraft pulp to whiteness is a difficult task, which when accomplished by the use of a hypochlorite bleach liquor is accompanied both by high bleach usage and marked injury to the papermaking characteristics of the fiber. The product of the 25 present invention, however, is one which is produced by a special processing of the kraft pulp aimed at the preservation of the valuable papermaking characteristics of such 30 pulp while removing from the pulp so much of its coloring matter and other constituents as are undesirable from the papermaker's standpoint. The product of the present invention is not one which is of extraordinarily 35 high alpha cellulose content, for if it be attempted to refine kraft pulp markedly in so far as concerns increasing its alpha cellulose content, it loses especially in such properties as strength, even though it may be improved 40 in other respects, such as softness and stability.

In producing the product of the present invention, I proceed as follows. A raw kraft pulp is subjected to the action of chlorine wa- 45 ter or to hypochlorite bleach liquor, or to a

succession of such reagents, without visible whitening of the pulp. In fact, the chlorine and/or hypochlorite should be used in such amount that the pulp after treatment has a distinctly different hue than the raw kraft 50 pulp. For example, raw pulp may be treated at temperatures of from 50° to 100° F. for two to six hours, as a 4% to 6% stock suspension in chlorine water containing 4% to 8% chlorine, based on pulp. During this treatment, the pulp assumes a deep orange color. The treated pulp is then washed free of treating reagent and reaction products. When 55 the washed pulp is tested, it exhibits a lower lignin content than that present in the original pulp. Ligneous matter is thus removed from the pulp without injury to its papermaking characteristics.

The washed pulp is then treated with an alkaline liquor similar to the cooking liquor 60 used in the kraft process of fiber liberation, namely, one containing both caustic soda and sodium sulphide. Preferably, the liquor is one containing 2% to 4% alkali, calculated as caustic soda equivalent, but 40% of which 65 alkali is present in the form of sodium sulphide. The pulp is suspended in this specific liquor as an 8% to 10% stock suspension at 50° to 70° C., for from one to four hours. During this treatment, the pulp is further 70 freed from lignous matter, but without impairing its papermaking characteristics. The pulp is then washed, at which stage it 75 has a lignin content of from 1% to 1.5%, as against a lignin content of from 5% to 7% in 80 the raw kraft pulp. It is thus seen that the process thus far is directed largely at the selective removal from the pulp of lignous matter, the initial treatment selectively removing some of the lignin and chlorinating 85 the rest, and the second treatment being conducted in an alkaline solution under conditions to dissolve out the chlorinated lignous matter. The selective dissolving out of the 90 chlorinated lignous matter, as already in-

dicated, takes place at particular temperature conditions in a solution containing particular amounts of both caustic soda and sodium sulphide. Such temperature conditions are conducive to the desired dissolving out action without the marked refining effect on the fiber which might be accomplished at higher temperatures or with a higher concentration of alkali in solution.

10 For instance, if the treatment of the pulp be carried out at higher temperature with the solution of alkali hereinbefore described, say 90° to 100° C. or higher, it is found that there is a marked sacrifice in the tear resistance of the pulp, even though its Mullen or pop strength is not appreciably affected. On the other hand, if the treatment of the pulp be carried out at temperatures lower than those specified with the solution of alkali hereinbefore described, there is a less effective removal of lignin from the pulp and a strong tendency to reduce the Mullen and tensile strength of the pulp; and there is apt to be an increase in the alpha cellulose content of the pulp to a point where it approaches the characteristics of a refined wood pulp. It is thus seen that the treatment of the pulp with a solution of alkali to produce the product of the present invention is conducted within a temperature range designed to effect an extensive elimination of lignin from the pulp without appreciably affecting its alpha cellulose content or its strength and tear resistance characteristics.

35 The alkaline-digested and washed pulp is now ready to be bleached. Bleaching, too, must be carried out in a special way, in order to arrive at my novel product. To this end, the pulp is subjected to a series of three independent bleaching treatments. The first two bleaching treatments consist in maintaining the pulp for three to six hours as a 5% suspension in hypochlorite bleach liquors at 70° F., —3% calcium hypochlorite based on pulp being used in the first treatment, 2% calcium hypochlorite based on pulp being used in the second treatment, and 0.5% caustic soda based on pulp being added to the bleaching liquors in each treatment. The 40 pulp is washed and thickened between the first two treatments, and again washed and thickened after the second treatment. The third bleaching treatment consists in maintaining the fiber for four hours as a 5% suspension in a permanganate solution at 70° to 75° F., containing about 0.3% potassium permanganate based on pulp. At the end of this treatment, the pulp is washed, but it 45 has a light tan color because of residual manganese oxides clinging to the fiber. The oxides are completely removed by treating the pulp with a dilute sulphurous acid solution and washing. The resulting product, 50 which is in pure-white condition, may be de-

livered to machines which form sheets ready for shipment.

The following table indicates the transformation effected upon the given kraft pulp in producing the product of the present invention:

|                     | Kraft   | Product of present invention |
|---------------------|---------|------------------------------|
| Color               | Brown.  | Pure white.                  |
| Total cellulose (%) | 90-93.0 | 98.5-99.5                    |
| Alpha cellulose (%) | 89      | 87-89                        |
| Cu. No.             | 1.2     | 1.0-2.0                      |
| Ash (%)             | .6-1.0  | 0.1-0.3                      |
| Resins (%)          | .2-.4   | 0.1-0.3                      |
| Pentosans (%)       | 7-9     | 3.0-5.0                      |
| Strength            | 150-160 | 150-160                      |
| Tear resistance     | 250-270 | 250-270                      |

It is to be observed that the product of the present invention, in addition to having the papermaking characteristics, including strength and tear resistance, of kraft pulp, is of pure-white color and has an extremely low resin content,—in fact being lower in resinous specks than most bleached sulphite pulps on the market. It has a much higher total cellulose content than the original pulp, but its alpha cellulose content is practically the same as that of the original pulp. Its pentosan content is somewhat lower than that of the original pulp, but there are sufficient pentosans therein in a form imparting toughness or strength to the sheet, without developing the brittleness imparted to a kraft pulp when it is whitened, for example, by successive treatments with sulphurous acid and hypochlorite bleach liquor.

While the product of the present invention has been described as being derived more especially from kraft pulp, it may be derived from other suitable alkaline-cooked wood pulps, for instance, the long-fibered soda pulps obtained by effecting fiber liberation from coniferous woods in so-called soda cooking liquors.

What I claim is:

1. A pure-white wood pulp derived from alkaline-cooked pulp as a raw material, possessing the strength and tear resistance of its derivation material, but being of lower pentosan and much lower resin content than its derivation material.

2. A pure-white wood pulp derived from alkaline-cooked pulp as a raw material, possessing the strength and tear resistance of its derivation material, being of lower pentosan and much lower resin content than its derivation material, and having a total cellulose content in excess of, but an alpha cellulose content only about equal to, its derivation material.

3. A pure-white wood pulp derived from kraft pulp as a raw material and having the following characteristics, to wit: (a) a total cellulose content of from 98.5% to 99.5%, (b) an alpha cellulose content of from 87% to 90%.

to 89%, (c) a copper number of from 1.0 to 2.0, (d) an ash content of from 0.1% to 0.3%, (e) a resin content of from 0.1% to 0.3%, (f) a pentosan content of from 3.0% to 5.0%,  
5 (g) and possessing the strength and tear resistance of the kraft pulp from which it is derived.

In testimony whereof I have affixed my signature.

10 GEORGE A. RICHTER.

15

20

25

30

35

40

45

50

55

60

65